

May 13, 1930.

A. KADOW

1,758,113

FORMING METAL CASTINGS

Filed March 15, 1926



Inventor

August Kadow.

By Owen & Owen

Attorneys

## UNITED STATES PATENT OFFICE

AUGUST KADOW, OF TOLEDO, OHIO, ASSIGNOR OF ONE-HALF TO WILBER OWEN AND CHARLES W. OWEN, OF TOLEDO, OHIO

## FORMING METAL CASTINGS

Application filed March 15, 1926. Serial No. 94,715.

This invention relates to casting, and more particularly to casting metal and compressing the metal in the casting while still hot.

The principal object of the invention is 5 to provide a method and apparatus by means of which a very dense casting may be made, and by which a selected surface portion may be condensed and smoothed. Minor objects 10 of the invention will appear as the description proceeds.

The invention will be described as applied to making cast bushings.

In the accompanying drawings, forming a part of this disclosure, Figure 1 is a somewhat diagrammatic vertical section through one form of apparatus suitable for casting bushings; Figs. 2 and 3 are sections on the same plane as Fig. 1, showing portions of the apparatus in successive stages of the operation; and Fig. 4 is an enlarged section on the same plane, showing the same parts as in Figs. 2 and 3, in a position which they assume during the final stage of the operation.

In carrying out my invention, a ladle 1, or 25 other suitable receptacle, is provided for molten metal 2. A mold 3, of suitable design, is brought into working relation with the molten metal, and the mold cavity is evacuated through suitable passages 4 leading to any 30 suitable means for exhausting air and other gases. Thereupon, the metal rises through inlet opening 5 and around plunger 6 to form a bushing 7.

Around plunger 6 and above the mold 25 cavity there is a sleeve 8. A spring 9 surrounds the sleeve and presses upward against a shoulder or flange 10 on the sleeve, normally raising the sleeve until the upper side of the flange contacts a cover plate 11.

40 The plunger has a head 12 and a fixed collar 13 between which there is a channel or groove 14. A plunger 15 of a suitable press is provided with clamping jaws 16 adapted to enter groove 14.

45 Plunger 6 is of a size to fit snugly within sleeve 8 and inlet opening 5. There is a reduced portion 18 extending from a shoulder 19, normally level with the bottom of sleeve 8, to a shoulder 20 at the lower end of the plunger. The amount of reduction of por-

tion 18 is exaggerated in the drawings for purpose of illustration. The normal position of plunger 6 is with its shoulder 20 slightly above inlet opening 5, so as to form a narrow inlet slot beneath the lower end of the plunger.

55 Preferably this inlet slot is narrow enough so that the mold and the source of supply of metal may be separated immediately after the mold is filled without the metal running back out of the mold by gravity. If desired, plunger 6 may be raised higher during filling, leaving a wider inlet slot, to expedite the filling action. In the preferred form, where 60 only a narrow inlet slot is used, plunger 6 may rest on sleeve 8 during the filling operation, as shown in Fig. 1, and a slight downward movement of both suffices to completely close the inlet, as shown in Fig. 2. If the 65 operation is such that some of the molten metal solidifies around the walls of inlet 5 and beneath the end of plunger 6, this metal, commonly called the "gate", is sheared off 70 from the casting when plunger 6 is lowered.

75 In the construction illustrated, lugs are provided on the sides of the mold, which are in front and back of the mold as viewed in Fig. 1, and so do not show. These lugs are rested upon firm abutments to support the mold when pressure is exerted by plunger 15, 80 and the mold is held firmly, by means not shown, against the spreading pressure of the metal in the mold cavity.

85 It will be understood, of course, that a container holding a comparatively large amount of metal may be used instead of the ladle shown, and that the pressing may take place with both container and mold in filling position, or that either container or mold or 90 both may be moved vertically, laterally or both between the filling and pressing operation. Where mold and container are separated between the filling and pressing steps, the mold may be supported from beneath instead of by lugs on its sides.

95 Preferably, pressure is exerted by plunger 15 while at least a portion of the metal in the mold cavity is liquid, and heavy pressure is used, amounting to many tons to the square inch, so that the metal in the mold cavity re-

maining liquid until pressure is applied is at once solidified by pressure raising the melting point, instead of being solidified by cooling. The pressure is maintained until the metal is sufficiently cool to remain solid when the pressure is removed. Where the metal is fairly near the point of solidification before the pressure is applied, and the loss of heat is fairly rapid, it is possible to lower and raise the pressing plunger with no appreciable pause at its lowest point, but in cases where the metal is hotter when pressure is applied and where loss of heat is comparatively slow, a dwell of the plunger at its lowest point, with pressure applied, is requisite.

Immediately after the mold is filled with metal, it is brought into operative relation to plunger 15, if not previously in line therewith.

When the casting has become solid, but while it is still very close to the melting point, the action of plunger 15 is reversed, and plunger 6 is drawn upward out of the casting. Sleeve 8 moves with plunger 6 until flange 10 encounters cover 11. Then movement of the sleeve is stopped and the plunger is pulled out of the casting. At first the casting moves upward with the plunger, leaving a space 23 between the bottom of the casting and the mold bottom equal to the amount the casting has shrunk under compression. Thereafter shoulder 20 is drawn up through the compressed and solidified casting 24, as shown in Fig. 4, still further compressing as well as smoothing and burnishing the interior surface portion 25.

Where desired, independent means may be provided for operating sleeve 8 and plunger 6, and the plunger might be provided with more than one broaching ring or shoulder, of successively greater diameters. If desired, such broaching rings might be provided on the plunger above the mold cavity, and the plunger might be driven down through the casting to broach it; but the arrangement shown is simpler, and is preferable where it satisfactorily performs the broaching and burnishing operation.

It will be understood that, where the nature of the finished article renders this desirable, a portion only of the interior of the article might be broached or burnished by sliding the corresponding portion of the plunger or mold-core therealong, and a similar burnishing action could be exerted upon all or any desired portion of the exterior of the casting by arranging a slide to form that portion of the mold surface and providing means for forcibly moving the slide with respect to the casting while it is still within the mold.

By evacuating the mold and introducing the metal in the manner described the mold is filled very quickly and with little entrapped air or gases. It is advantageous to fill the

mold quickly, so that the entire casting may be of approximately the same temperature when pressure is applied, and absence of air or gas reduces the openings or pores in the metal. It is frequently desirable to coat some or all of the surfaces of the mold cavity with a poor conductor of heat, to avoid too rapid chilling of the casting.

The subjection of the metal to heavy pressure while setting prevents it from shrinking away from the mold walls or plunger upon solidification, maintains intimate contact between the metal of the casting and the mold wall and so hastens transfer of heat and consequent cooling of the casting, and tends to prevent the formation of pores or openings in the metal and closes those which do form, thus producing a very dense and uniform casting of the exact thickness determined by the spacing of the mold wall and plunger.

The final withdrawal of the plunger, with the broaching and burnishing action of shoulder 20, while the metal is still close to the molding point, insures that, when the casting is completed, its bore will be uniformly of the exact size determined by said shoulder, and that the surface of the bore will be exceedingly dense and smooth, a result particularly desirable in bushings.

Most metals contract upon solidifying. The contraction is especially marked in lead and in alloys containing a considerable percentage of lead, but it occurs in other metals. Where a liquid contracts upon solidification, the melting point is raised by pressure. For that reason, when metal in a mold is liquid near the solidifying temperature, or partially liquid and partially solid, heavy pressure raises the melting point and solidifies, or completes solidification of, the metal, as mentioned above. When the solidification takes place because of pressure sufficient to raise the melting point above the temperature of the previously liquid metal, it is obvious that the mold cavity is completely filled upon solidification, and therefore contraction of the casting away from the mold walls due to shrinkage in solidification is eliminated.

Of course, the solidified casting continues to cool after plunger 6 is withdrawn, and shrinks while cooling. If the apparatus is manipulated so that plunger 6 is withdrawn at such times as to leave the castings at a substantially uniform temperature, this shrinkage is uniform, and the diameters of the bores of the finished article are likewise uniform.

When metal is solidified by cooling, it tends to shrink in every direction, and so opens up or enlarges pores throughout its structure. When metal is solidified by pressure, there is a tendency to reduce the size of any pores caused by gas, and to prevent the separation of occluded gas to form bubbles and open up pores.

Immediately after setting, and while still

very hot, the metal in the casting yields to pressure, so that heavy pressure brought to bear upon the casting in the mold immediately after setting fills out the mold cavity and reduces the size of pores in the metal. Thus, some of the benefits of my process may be realized when the metal is allowed to solidify before pressure is exerted. A pressure insufficient to raise the melting point of the metal above the temperature at which it is subjected to the pressure may be sufficient to condense the metal somewhat and improve its quality, and thus some of the benefits of my process may be obtained when the degree of pressure applied or the temperature of the molten metal to which it is applied is such that the metal is not immediately solidified. But there is a tendency for occluded gases to separate and form bubbles as the metal cools, whether or not it is under pressure, and there is a tendency for impurities in metals and ingredients in alloys to segregate to some extent and destroy the uniformity of the casting when it cools and solidifies gradually. For the best results, therefore, it is best to apply to the still molten metal a pressure high enough to solidify it.

It is old to burnish metal by rubbing it, generally without materially displacing the surface. A similar, but more effectual, action results when the metal is hot and the rubbing displaces the surface and condenses an appreciable layer as well as smoothing the surface skin.

The shape of the mold, the shape, size and method of moving pressing plungers and burnishing slides, the material of which various portions of the mold are made, the thickness of the mold walls, coatings of desired kinds on portions of the mold cavity, the temperature at which the metal is drawn into the mold, the degree and duration of pressure, and various other details may be varied in accordance with the metal which is being cast and the size, shape and other desired qualities of the object being formed.

I claim:

1. The process which consists in withdrawing air from one end of a mold chamber, introducing molten metal into the other end of the chamber, and, while the introduced metal is still hot, exerting pressure against the metal in the first said end and in a direction towards the second said end.

2. The process which consists in evacuating a mold cavity and filling it with molten metal, closing the mold and, while a portion of the metal in the mold is still molten, moving a portion of the molding surface of the cavity inward to press said metal.

3. The process which consists in filling a mold with molten metal, while the metal is at least partially molten, subjecting it to pressure sufficient to raise its melting point and complete its solidification, and maintaining

the pressure until the casting is cooled below its normal melting point.

4. The process of producing castings in a mold having relatively movable sections, which consists in evacuating air from the mold through a joint between its sections, filling the mold cavity with molten metal and thereafter pressing the metal in the cavity by moving one of said sections inward along said joint and reducing the size of the cavity.

5. The process which consists in evacuating a mold chamber and filling the chamber with molten metal, while the metal is at least partially molten subjecting it to pressure sufficient to raise its melting point and complete its solidification, and maintaining the pressure until the casting is cooled below its normal melting point.

6. The process which consists in casting metal in a mold and burnishing a portion of the surface of the casting by movement of a portion of the mold wall with respect to the casting.

7. The process which consists in casting metal and burnishing by rubbing pressure a portion of the surface of the casting after it has solidified and while it is still near its melting point.

8. The process which consists in evacuating a mold chamber, filling the chamber with molten metal and forming a casting and burnishing by rubbing pressure a portion of the surface of the casting after it has solidified and while it is still hot.

9. The process which consists in filling a mold chamber with molten metal, compressing the metal in the chamber, and after the metal has solidified into a casting, but while it is still hot, burnishing a portion of the surface thereof.

10. The process which consists in evacuating a mold chamber and filling it with molten metal, solidifying the metal in the mold by compression, and burnishing a portion of the surface of the metal while it is still hot.

11. The process of forming a bushing, which consists in filling an annular space in a mold with molten metal and subjecting the metal, before cooling, to pressure longitudinally of its axis heavy enough to reduce its volume.

12. The process of forming a bushing which consists in filling an annular space in a mold with molten metal, subjecting the metal, before it has completely solidified, to pressure sufficient to raise its melting point and complete its solidification, and maintaining the pressure until the metal has cooled sufficiently to retain its solid state when the pressure is removed.

13. A process in accordance with claim 7, in which the pressure is applied longitudinally of the axis of the bushing.

14. The process of forming a bushing which consists in casting a bushing and, while

70

75

80

85

90

95

100

105

110

115

120

125

130

it is still hot, burnishing its interior surface.

15. The process of forming a bushing, which consists in casting a bushing and, while it is still hot, broaching and burnishing its interior surface.

16. The process of forming a bushing which consists in casting a bushing, and compressing the metal in the casting longitudinally and broaching and burnishing its interior surface while it is still hot.

17. The process which consists in casting a bushing about a plunger having an enlarged end and, while the bushing is still hot, broaching and burnishing it by forcing the enlarged end of the plunger therethrough.

18. The process which consists in casting a bushing about a plunger having an enlarged end, compressing the casting about the plunger, and thereafter broaching and burnishing the casting by forcing said enlarged end of the plunger therethrough.

19. The process which consists in filling molten metal into an annular space about a plunger having an enlarged end, exerting pressure upon the metal before it is fully solidified, compressing it about said plunger and raising its melting point to complete the solidification thereof, and thereafter broaching and burnishing the casting by forcing said enlarged end therethrough.

20. The process of forming a bushing, which consists in positioning a permanent mold, about a plunger having an enlarged end, so that an inlet slit is left between said enlarged end and the mold wall, evacuating the mold and filling it with molten metal through said slit, and thereafter moving said enlarged end to close the slit and shear off the gate.

40 21. The process of forming a bushing, which consists in positioning a permanent mold, having an annular casting space, about a plunger having an enlarged end, so that a slit is left between one end of said mold space and said enlarged end, evacuating said annular space and introducing molten metal through said slit to fill said space, thereafter moving said enlarged end to close said slit and compressing the metal in said space longitudinally, and thereafter, while the said metal is still close to the melting point, broaching and burnishing the opening therein by passing said enlarged end therethrough.

55 22. In casting apparatus, a mold having a casting space therein, a plunger extending through the said space, a collar surrounding the plunger, and means to move said collar to compress the metal in said space.

60 23. In casting apparatus, a mold having a casting space therein and passages through which gas may be evacuated from said space, a plunger extending through the said space, a collar surrounding the plunger, and means to move said collar to compress the metal in said space.

24. In casting apparatus, a mold having a casting space therein, a plunger having an enlarged head, and means to move said plunger and reciprocate its head completely through said space.

70 25. In casting apparatus, a mold having a casting space and an inlet opening, a plunger adapted to extend through said space, a sleeve surrounding said plunger, the end of the sleeve forming a portion of the wall of said space, yielding means normally holding the sleeve in a predetermined position, connections between the sleeve and plunger adapted to hold the plunger with its end adjacent the inlet opening when the sleeve is in said position, and means for forcing the plunger and sleeve towards said inlet.

75 26. In casting apparatus, a mold having a central bore shouldered at one end to form a reduced inlet opening, a sleeve in the other end of the bore having an opening the same size as said inlet, and a plunger extending through said sleeve to said inlet.

80 27. In casting apparatus, a mold having a bore therethrough, a plunger working in said bore, and an annular casting space surrounding the plunger, the plunger being slightly reduced in cross section where it is normally in register with the casting space.

85 28. In apparatus in accordance with claim 20, a sleeve filling a space between the plunger and walls of the mold bore at an end of said bore, the inner end of the sleeve forming one end of the casting space.

90 29. In casting apparatus, a mold having a central bore therethrough and evacuating passages leading from said bore, the bore being reduced at one end to form an inlet opening, a plunger entering the other end of said bore, and means normally holding the end of the plunger spaced slightly from the inlet opening leaving a narrow slot between the end of the plunger and the shoulder where the bore is reduced to form said inlet opening.

95 30. In casting apparatus in accordance with claim 22, a sleeve surrounding the plunger, a spring exerting outward pressure on the sleeve, a stop to limit the outward movement of the sleeve, and a collar on the plunger adapted to limit the inward movement of the plunger with respect to the sleeve.

100 31. In casting apparatus, a mold having a vertical bore reduced at its lower end to form an inlet opening, evacuating passages leading into said bore, a stop plate on the upper end of the mold, a sleeve in the upper end of the bore, a spring adapted normally to raise the sleeve against the stop plate, a plunger within the sleeve, a collar on the plunger in position to rest on the upper end of the sleeve when the lower end is spaced slightly above the inlet, the plunger being adapted to fit within the sleeve, the lower end of the plunger being adapted to fit within the inlet opening and the diameter of the plunger being

70

75

80

85

90

95

100

105

110

115

120

125

130

slightly less above said lower end up to even with the normal position of the bottom of the sleeve, and means for reciprocating said plunger.

<sup>5</sup> In testimony whereof, I have hereunto signed my name to this specification.

AUGUST KADOW.

10

15

20

25

30

35

40

45

50

55

60

65